

Aug. 22, 1933.

L. T. TROLAND

1,923,764

PHOTOGRAPHIC GELATIN RELIEF

Filed Jan. 30, 1931

*Fig. 1.*



*Interchangeable*



*Fig. 2.*

Travertor  
Leonard L. Troland  
By Roberts, Cushman & Woodbury  
his attorneys.

## UNITED STATES PATENT OFFICE

1,923,764

## PHOTOGRAPHIC GELATIN RELIEF

Leonard T. Troland, Cambridge, Mass., assignor,  
by mesne assignments, to Technicolor, Inc.,  
New York, N. Y., a Corporation of Delaware

Application January 30, 1931. Serial No. 512,398

12 Claims. (Cl. 95—5.6)

In the photographic art two main processes are known for making photographic gelatin reliefs from silver halide emulsions. One process involves the use of developers which harden the exposed parts of a silver halide emulsion, as for instance the well-known pyrogallic developer. The other process involves the developing of the latent image with an ordinary non-hardening developer, as for instance a sulphite-containing 5 metol-hydroquinone developer, and the subsequent hardening of the developed image with selectively hardening agents, as for instance an acid solution of bichromate. Although developer hardened reliefs are comparatively rugged, durable and easy to make, the reliefs made by the second method are preferable for certain purposes, especially for making motion picture positives, because they have a finer grain structure and a better photographic characteristic than reliefs made with hardening developers. However, the method using a separate hardener has two disadvantages which impair its practical application. If the non-hardening developer is not thoroughly washed out before the emulsion has 10 passed into the independent hardener, there is a tendency towards a general hardening of the entire emulsion layer containing the remainder of the developer, so that the unaffected parts of the emulsion, which has been exposed through its support, can not be removed in the subsequent hot water bath, the so-called etch, and no relief can be obtained. On the other hand, if the developing agent is completely removed by a thorough washing, the relief tends to disintegrate in the subsequent hot water bath. It is very difficult to balance these two actions by adjusting the washing bath, in order to prevent too much hardening and/or disintegration of the relief. 15 The main object of the present invention is therefore to provide a photographic gelatin relief which has the desirable properties of a relief obtained by independently hardening the developed image, and which can be manufactured as easily as reliefs made with hardening developers. Another object is to provide a photographic process for making gelatin reliefs of a structure, and with characteristics suitable for certain purposes such as motion pictures, which can be easily carried out on a commercial basis. Still another object is to provide a development which controls and stabilizes the hardening action of a subsequently applied independent hardening agent. A further object is to provide a new 20 hardening process for gelatin reliefs which com-

bines the advantages, while avoiding the disadvantages, of the two known main processes for making such reliefs. Other objects will be apparent from the following description of the invention which is accompanied by a drawing, in 25 which

Fig. 1 shows the structure of a photographic emulsion treated according to the present invention; and

Fig. 2 is a flow sheet of the process according 30 to the invention.

In order to overcome the difficulties outlined above, the process according to the present invention combines an ordinary non-hardening development with a hardening development and with 35 separate hardening, thereby obtaining a relief which has the desirable properties of the separately hardened relief without the disadvantages of the process for making such reliefs. Superficially it might appear that no advantage could 40 be gained by combining these processes, but experiments have shown that a distinct improvement of the gelatin relief can be obtained if the processes are combined. The treatment in a hardening developer hardens the image to a degree which prevents its disintegration during the thorough washing required to remove all the developer which otherwise might result in hardening more than the exposed parts of the emulsion 45 in the subsequent bath in a differential hardener. Moreover, there is a certain cooperation between the residues of the hardening development and the independent hardener. For the purpose of a better understanding of the invention, the separate actions of hardening developers, for instance 50 pyrogallic, and of independent hardeners, for instance chromic acid, will first be explained.

After development in a hardening developer each silver grain is surrounded by a hardened zone of considerable size in comparison with the grain. The hardness of this zone depends upon the concentration of the developer and the time allowed for its action. The gelatin zone surrounding the emulsion particles may become sufficiently 55 hard so that subsequent etching (after the non-hardened gelatin, corresponding to unexposed parts, is dissolved by the warm water), will leave a gelatin relief. If the hardening is carried on far enough all silver grains, which are connected by hardened zones to each other and to the base, contribute to the relief and only those which have no connection whatsoever are etched off. However, if the hardening is carried on to such a degree a noticeable grain appears upon the surface of the 60 relief and imparts thereto a pattern in addition 65

to that which forms the picture, which is very undesirable. If the development is not carried on far enough to produce this effect many insufficiently hardened portions are lost and the relief 5 does not truly reproduce the original photographic image. In either case the developed zones contain certain oxidation products of the hardening developer and the size of these zones do not correspond with the concentration of the developer, 10 the concentration controlling the hardness of the zone rather than its size.

Considering now the independent hardening, a chromic hardener is reduced by the silver image and produces hardened zones surrounding the 15 grains. In the commonly used and commercially feasible chromium hardening process these zones are substantially confined to gelatin parts immediately surrounding the grains, are therefore considerably smaller than the corresponding zones 20 produced by a hardening developer, and the subsequent etching in warm water will remove quite a considerable number of gelatin particles which have no connection with each other nor with the base. On the other hand, the surface pattern of 25 a gelatin relief made in this manner is very much less pronounced than that of a developed relief and such a relief is therefore much better suited for certain purposes (as e. g. for imbibition printing from the relief) than a developer hardened 30 relief.

My improved process permits the making of a relief having these desirable properties without incurring the aforesaid disadvantages of the separate hardening method. This new process will 35 first be described in connection with an explanation of its beneficial action, based upon a theory of the process which appears to be the most plausible one in the light of investigations available at the present time. Directions for carrying 40 out the process will then be given as one of the possible practical embodiments of the invention.

The exposed emulsion consists of grains of various sizes, as shown in the drawing. This emulsion is first treated in an ordinary non-hardening developer. As known in the art the reducing action of a developer starts at points near the surface of the larger particles of exposed silver and spreads from there gradually over the whole particle. Considering the particle 1 45 (Fig. 1) for example, the non-hardening developer starts to reduce the particle at 2 and from there the action continues until the stippled part 3 of the grain is reduced to metallic silver. The development with the non-hardening developer is 50 interrupted at this stage of the process, and continued with a hardening developer. This will now finish the development of the larger particles, but also reduce the small particles 4, which have not yet been attached by the first developer, and 55 zones surrounding both the remainder of the larger particles, of about the size of the smaller grains, and the smaller grains themselves will be thoroughly hardened by the second developer. At this stage of the process there are larger zones 60 of unhardened gelatin containing metallic silver, and smaller zones of hardened gelatin, also containing metallic silver, which surround the unhardened zones thereby protecting them and cementing them together so that the emulsion will 65 not disintegrate during the now following step of removing the developer thoroughly from the emulsion by washing. An initial development in a hardening developer followed by a bath in a non-hardening developer has practically the same 70 effect, as will be obvious to anyone skilled in the

art. The next step is the separate hardening with a chromium compound with hardens the remaining unhardened zones containing reduced silver. It is probable that the residuary oxidation products of the hardening developer penetrate even beyond the developer hardened zones, and these oxidation products react with the independent hardener, which results in an independent tanning action similar to and augmenting that caused by the silver at 3, which was reduced by the non-hardening developer. The emulsion is then treated in warm water, which dissolves all unhardened parts of the gelatin. 80

During the etching process, practically the whole emulsion as far as it was influenced by light will be preserved because the chromate hardened parts, which would normally not extend beyond the zones of reduced silver and therefore tend to disintegrate, are cemented together by the developer hardened zones corresponding to the small exposed silver halide particles and because the action of the independent hardener is extended due to the oxidation products of the hardening developer which penetrate beyond the developer hardened zones. Accordingly, the surface of the relief will substantially have the character of a chromium hardened relief, since its larger part consists of gelatin hardened with chromium, whereas the developer hardened zones of the surface are too small to cause undesirable 105 irregularities of the relief surface. It is of course understood that the final product will not contain metallic silver, because the customary chromic hardeners are also bleaching agents. The remaining silver bromide is removed in a 110 customary thiosulphate fixing bath.

The following exact directions for carrying out my new process in one of its preferred embodiments are given by way of example.

The exposed emulsion is first developed in a 115 developer made according to the following formula:

|                                                  |            |     |
|--------------------------------------------------|------------|-----|
| Metol (monomethyl paraaminophenol sulphate)----- | 3.1 grams  | 120 |
| Sodium sulphite-----                             | 45.0 grams |     |
| Hydroquinone-----                                | 12.2 grams |     |
| Sodium carbonate-----                            | 67.5 grams |     |
| Potassium bromide-----                           | 1.9 grams  | 110 |
| Water to-----                                    | 1 liter    | 125 |

This developer should have a temperature of approximately 68° F., and the film should remain therein for about three minutes and twenty seconds. After a washing sufficient to remove any constituents of the first developer not desired in the second bath, the film is removed into the hardening developer of the following composition:

|                        |           |     |
|------------------------|-----------|-----|
| Pyrogallic acid-----   | 8.2 grams | 130 |
| Citric acid-----       | 0.2 grams |     |
| Potassium bromide----- | .40 grams |     |
| Sodium hydroxide-----  | 3.4 grams | 140 |
| Ammonium chloride----- | 1.7 grams |     |
| Water to-----          | 1 liter   |     |

This formula corresponds to the developer formula as disclosed in my United States Patent No. 1,535,700 of April 28, 1925, and was found to give satisfactory results also if used in the process according to the present invention. The film is then washed for approximately five minutes and forty seconds in water of approximately 68° F. 150

The film is then removed to a bath of the following composition:

5. Chromic acid ..... 5 grams  
Sodium chloride ..... 25 grams  
Water to ..... 1 liter

After having been removed from this hardening bath, the unhardened parts of the emulsion are brought into a water bath of about 130° F., and then dried for about twelve minutes at 100° F.

10. in which the film remains for about four minutes.

After this the film is fixed for about two minutes in the customary fixing bath of about 69° F., and then in alcohol of 68° F., also for one minute, and then dried for about twelve minutes at 100° F.

15. It is of course understood that other hardening and non-hardening developers and various independent hardeners can be used and that the proportions of the ingredients and the exact directions for the steps of the process may be

20. varied in accordance with the properties of different agents acting generally in the same manner as the agents expressly mentioned above. For instance, a pyrogallol developer containing sufficient sulphide to prevent any hardening action

25. can be used instead of the metol developer or another inherently non-hardening developer, a pyrocatechol developer may be used instead of pyrogallol and acidic bichromate can be used instead of chromic acid.

30. It should also be understood that the present disclosure is for the purpose of illustration only and that this invention includes all modifications and equivalents which fall within the scope of the appended claims.

35. I claim:

1. The method of making photographic gelatin reliefs which comprises partly developing an exposed silver halide emulsion in a solution containing substantially non-hardening reducing

40. agents, partly developing said emulsion with a gelatin hardening reducing agent and subsequently selectively hardening the developed silver image.

2. The method of making photographic gelatin reliefs which comprises partly developing an exposed silver halide emulsion in a non-hardening developer containing hydroquinone, partly developing said emulsion in a pyrogallol developer and then bleaching and hardening the developed

50. image in a chromic acid solution.

3. The method of making photographic gelatin reliefs which comprises partly developing an exposed silver halide emulsion in a solution containing approximately 3 grams metol and 45

55. grams sodium sulphite in 1 liter of water, partly developing said emulsion in a solution containing approximately 3.2 grams pyrogallic acid and 3.4 grams sodium hydroxide in 1 liter of water, washing the emulsion, hardening the emulsion in a

60. solution containing approximately 5 grams chromic acid and 25 grams sodium chloride in 1 liter of water, and removing the unhardened portions of the emulsion.

4. The method of making photographic gelatin reliefs which comprises developing and partially hardening an exposed silver halide emulsion in consecutive baths of non-tanning and tanning reducing agents, and subsequently hardening the developed silver image in a separate hardening solution.

5. The method of making photographic gelatin reliefs which comprises partly developing the latent image of an exposed silver halide emulsion

in a solution containing substantially non-hardening reducing agents, partly developing said emulsion with reducing agents hardening the gelatin sufficiently to prevent disintegration of the exposed portions of the emulsion but not sufficient to harden said portions completely and subsequently forming a relief image by completely hardening said portions with a differentially hardening bath and removing the unhardened portions.

6. The method of making photographic gelatin reliefs which comprises partly developing an exposed silver halide emulsion in a non-hardening developer, partly developing in a developer containing agents restraining subsequent disintegration of the gelatin forming the image and selectively hardening the developed image in a separate hardening solution.

7. The method of making photographic gelatin reliefs by developing the latent image of an exposed silver halide emulsion in baths of non-hardening and hardening developers but confining the hardening to developed portions, which comprises preliminary hardening of said portions together with completely developing them and total hardening of said portions in a differentially hardening solution.

8. The method of making gelatin reliefs which comprises partly developing an exposed silver halide emulsion in a substantially non-hardening developer, further developing said emulsion in a hardening developer producing oxidation products incidentally to development, and subsequently treating the emulsion in a hardening bath selectively controlled by the developed silver as well as said oxidation products.

9. The method of making gelatin reliefs comprising partly developing an exposed photographic emulsion in a solution containing substantially non-hardening reducing agents in combination with a subsequent complete development with reducing agents sufficiently hardening to preserve the exposed emulsion during subsequent treatment and completely hardening said emulsion with a subsequently applied independent hardener.

10. The method of making photographic gelatin reliefs which comprises partly developing the larger grains of the emulsion in a non-hardening developer, developing the smaller grains and the previously undeveloped portions of the larger grains in a hardening developer, and subsequently hardening in an independent hardening agent.

11. The method of making photographic gelatin reliefs which comprises partly developing the larger grains of the emulsion in a hardening developer, developing the smaller grains and the previously undeveloped portions of the larger grains in a non-hardening developer, and subsequently hardening in an independent hardening agent.

12. The method of making photographic gelatin reliefs which comprises developing comparatively large portions of the larger grains of the exposed parts of a photographic emulsion in a non-hardening developer, developing and tanning the remainder of the larger grains and the smaller grains in a hardening developer, and hardening said large portions in an independent hardening agent.

LEONARD T. TROLAND.